

## UNITED STATES PATENT OFFICE

2,018,752

## ALLOY

Richard R. Walter, Starnberg, Germany

No Drawing. Application May 7, 1929, Serial No. 361,263. In Germany December 3, 1928

7 Claims. (Cl. 75—1)

My invention pertains to alloys and more particularly to an alloy of tungsten carbide with some other metal of lower melting temperature or with a plurality of metals of the iron and 5 chromium groups respectively.

The tungsten carbides are extensively used in tools because of their great hardness and resistance to wear. Owing to their high melting temperature they are mostly sintered together 10 in powdered form by the addition of metals of lower melting temperature. It is known that the metal or metals to be added for reducing the temperature of the sintering process should not exceed ten or at the most twenty per cent else 15 the alloy will lose its character and particularly its requisite hardness.

The tungsten carbide alloys uniformly manifest a certain brittleness which in many cases 20 greatly delimits their field of usefulness, consequently, further to increase the additions of other metals, which are adapted to lessen brittleness, seemed corrective, but did not prove so because of the falling off in hardness which hitherto occurred.

Accordingly, one object of my invention has 25 been to produce a cutting and wear-resisting alloy which will more successively combine the hardness property of the carbide with the added strength lent by another metal or metals. A further object has been successfully to increase 30 the proportion of metal or metals to be alloyed with the carbide or with a carbonitride of a metal of the chromium group. The new and useful function of carbonitrides in this particular art 35 is set forth and claimed in my copending application filed March 6, 1928, Serial No. 259,605.

Contrary to previous knowledge, I have discovered that tungsten carbide WC with six and 40 twelve-hundredth per cent (6.12%) C permits of substantially greater additions of metals adapted to improve the toughness and resistance to wear without unpermissible loss of hardness and that the presence of free or elemental tungsten amongst the auxiliary metals operates to especial 45 advantage. While the sintered tungsten carbides of at least eighty per cent (80%) of carbide content hitherto permitted an employment of alloyed metals of not more than twenty per cent (20%); according to the present invention, the metals to be alloyed with the tungsten carbide 50 may amount to fifty per cent (50%) of the latter and yet attain the desired increase in toughness and resistance to wear while remaining hard enough.

It was discovered that the amount of free tungsten in my alloy (agreeable to its purpose) should not be much less than five per cent (5%) and that more than thirty per cent (30%) of tungsten does not produce an improvement in quality. 5

I discovered furthermore, that the tungsten carbide can be successfully replaced with tungsten-carbonitride (W<sub>x</sub>C<sub>x</sub>N<sub>x</sub>) or mixed with the latter. These complex combinations manifest a substantial increase in mechanical strength as 10 compared with the carbides of greatest hardness and their resistance to wear exceeds that of the pure carbides.

The nitrification is facilitated and possible even with the metal tungsten if effected subsequent to 15 or simultaneous with a carburization, either while glowing in pulverized carbon or in the presence of heat through transition of hydrocarbons and while exposed to dissociated nitrogen.

As auxiliary or alloyed metals, besides the 20 tungsten content, one may use most of the metals of the iron and chromium groups (Fe, Mn, Ni, Co, and Cr, W, Mo, U respectively) either singly or several together. The carbides of the metals of these two groups are employed to advantage. 25 As is known, a small addition of boron can enhance the degree of hardness where that is desired.

The production of this alloy involves the usual method of pressing together the pulverized ingredients followed by sintering in a nonoxidizing atmosphere. The sintering temperature is generally below twenty-seven hundred and thirty-two degrees Fahrenheit (2732° F.) and the commencement of the sintering is ordinarily under 30 twenty-five hundred and fifty-two degrees Fahrenheit (2552° F.). 35

For example, one alloy embodying this invention and which manifests especially good cutting performances as a machining tool is composed of 40 the following combination:—

Sixty per cent (60%) WC

Twenty-six per cent (26%) W

Twelve and one-half per cent (12.5%) Co

One and one-half per cent (1.5%) Cr<sub>3</sub>C<sub>2</sub>

By utilizing a tungsten carbonitride one obtains a lathe tool alloy of exceptionally good cutting qualities, for example, with the following combination.

Fifty-nine per cent (59%) WC

Thirteen per cent (13%) 2WC<sub>1/2</sub>W<sub>3</sub>N<sub>2</sub>

Eighteen per cent (18%) W

Ten per cent (10%) Co

The nitrogen content of the carbonitride is 55

suitably controlled so that, for instance, in a machining tool the amount of nitrogen in the complete alloy is less than one per cent (1%), whereas for other purposes, when great hardness is the primary desideratum, the nitrogen proportion may be greater.

All the alloys embraced by this invention likewise find advantageous application where it is desirable to offer great resistance to impairment or loss by service, for example, in pulling tools, dies, bearing blocks or pivots or sockets and moreover for earth and mineral drilling tools and allied duty.

It is to be realized that the scope of my invention comprehends other equivalent methods and combinations and that the particular description declares only a few specific exemplifications of an extensive series of successfully feasible combinations each modified according to the character of service for which trial has established them to be best adapted, respectively.

I claim:

1. A sintered alloy comprising mixtures of tungsten carbide and tungsten carbonitride together with addition of metals of the iron and chromium groups characterized in that tungsten carbide and tungsten carbonitride together as the chief component constitute at least fifty per cent and less than eighty per cent.

2. An alloy comprising less than eighty per cent of a carbide of a metal of the chromium group, about ten per cent of a metal of the iron group and of the same metal as that of which the carbide is formed a per cent ranging from one-fourth to nearly one-half of the per cent of its carbide.

3. A sintered alloy comprising over fifty per cent of a carbide of a metal of the sixth periodic group, up to thirty per cent of a metal element of the sixth periodic group and as remainder a metal of the iron group.

4. A sintered alloy consisting of chromium carbide between 50 to 60%, tungsten between 15 to 20%, and an iron group metal as remainder.

5. A sintered alloy consisting of 78 to 80% tungsten, 6 to 20% of an iron group metal, and 2 to 3% carbon, the tungsten being in the form of tungsten carbide and metallic tungsten.

6. A sintered alloy comprising a carbonaceous compound of a metal of the chromium group between 50 to 60%, the same metal in elemental form between 15 to 20% and as remainder, metal of the iron group.

7. A sintered alloy comprising tungsten carbide over fifty per cent, elemental tungsten between somewhat less than 5 to 30% and metal of the iron group as remainder.

RICHARD R. WALTER.